

## UNITED STATES PATENT OFFICE

2,132,116

## ALLOY

Henry R. Kiepe, Newark, N. J., assignor to Baker & Company, Inc., a corporation of New Jersey

No Drawing. Application January 29, 1938,  
Serial No. 187,660

4 Claims. (Cl. 75—172)

This invention relates to alloys of which palladium constitutes the major portion, one object of the invention being to provide such an alloy which shall be harder than palladium, which can 5 be highly polished, which can be easily worked into various shapes, which shall have an attractive white color and shall be highly resistant to oxidation, tarnish or other discoloration.

Palladium is known to be a relatively soft 10 metal in both the annealed and the hard-worked state. It is also known that palladium can be hardened by alloying it with ruthenium. However, the structure of alloys of palladium and ruthenium is not good; there is a tendency of 15 the constituents to resist the formation of a uniform crystalline structure, as the result of which the harder or richer ruthenium particles appear as streaks in the alloy, especially when the alloy is polished. Moreover, the palladium-ruthenium alloys become practically unworkable 20 if they contain over ten percent (10%) of ruthenium.

I have discovered that these deficiencies of the palladium-ruthenium alloys can be eliminated or diminished by the addition of copper to 25 the palladium and ruthenium. The copper acts as a mutual solvent for the palladium and ruthenium, and thereby makes possible an alloy of uniform structure. These alloys containing sub- 30 stantially palladium, ruthenium and copper also are hard but not brittle, will take a high polish, resist oxidation and tarnish, and are easily workable. Therefore, they can be made into many different articles of simple or complicated shapes, 35 for example articles of jewelry, pen nibs, electric switch contacts, spinnerets used for manufacture of artificial silk, electrical resistance wires, dental and orthodontic appliances, and so forth.

40 As above stated, the alloy of the invention is predominantly palladium, the remainder being substantially ruthenium and copper. The proportions of the constituent metals may be widely varied. The amount of palladium, preferably, is 45 from eighty percent (80%) to ninety-eight percent (98%). The ruthenium content may be as low as five-tenths of one percent (0.5%) or as high as fifteen percent (15%), but preferably lies within the range of from one percent (1%) to ten percent (10%). The content of the copper 50 may similarly vary from five-tenths of one percent (0.5%) to fifteen percent (15%), but preferably the variations lie within the range of from one percent (1%) to ten percent (10%).

55 The particularly preferred alloy comprises sub-

stantially about ninety-three and one-half percent (93.5%) of palladium, about three and one-half percent (3.5%) of ruthenium and about three percent (3%) of copper.

A striking feature of the invention is the discovery that the deficiencies of the known palladium and ruthenium alloys can be overcome or reduced by the addition of copper to the palladium and the ruthenium. This remarkable effect of copper is demonstrated particularly in connection with the hardness of the alloys. Heretofore, alloys of palladium and ruthenium have been considered to be unworkable when more than ten percent (10%) of ruthenium is present. Copper is generally considered to be a 5 hardening agent, and ordinarily the addition of a hardening element to an alloy renders the resultant alloy still more difficult to work. However, I have discovered that the addition of copper to palladium-ruthenium alloys, makes the 10 resultant alloy more easily workable, even to the extent of making workable such an alloy containing as much as fifteen percent (15%) of ruthenium.

The following table illustrates the hardness 15 of various alloys lying within the scope of the invention.

| Pd<br>Percent | Ru<br>Percent | Cu<br>Percent | Brinell<br>(Baby Brinell 2<br>mm. ball, 120 kg.<br>load) |                                    |
|---------------|---------------|---------------|----------------------------------------------------------|------------------------------------|
|               |               |               | Hard<br>worked                                           | Annealed<br>1000° C. 15<br>minutes |
| 98            | 1             | 1             | 109                                                      | 59                                 |
| 95            | 4             | 1             | 158                                                      | 89                                 |
| 93.5          | 4.5           | 2             | 175                                                      | 107                                |
| 95            | 2             | 3             | 123                                                      | 74                                 |
| 93.5          | 3.5           | 3             | 163                                                      | 90                                 |
| 80            | 10            | 10            | 227                                                      | 166                                |
| 70            | 15            | 15            | 237                                                      | 152                                |
| 84.5          | 0.5           | 15            | 178                                                      | 101                                |
| 84.5          | 15            | 0.5           | 229                                                      | 198                                |

It will thus be seen that my invention provides 45 a novel and improved alloy which has the desirable precious metal characteristics of palladium and ruthenium, which has a beautiful white color, which is hard but not brittle, which is capable of being highly polished, which is resistant to oxidation and tarnish, and which is easily workable into many different articles requiring all or any of the aesthetic, physical, metallurgical and chemical properties hereinbefore 50 described.

5

10

15

20

25

30

35

40

45

50

55

Having thus described my invention, what I claim is:

1. An alloy containing from one-half of one percent (0.5%) to fifteen percent (15%) ruthenium and from one-half of one percent (0.5%) to fifteen percent (15%) of copper, the remainder being palladium.
- 5 2. An alloy containing ninety-three and one-half percent (93.5%) palladium, three and one-half percent (3.5%) ruthenium and three percent (3%) copper.

3. An alloy containing from one percent (1%) to ten percent (10%) ruthenium, and from one percent (1%) to ten percent (10%) copper, the remainder being palladium.

4. An alloy of palladium, ruthenium and copper wherein there is from eighty percent (80%) to ninety-eight percent (98%) of palladium, the remainder consisting of approximately equal amounts of ruthenium and copper.

5

10

HENRY R. KIEPE.